

1

3,192,073

**METHOD OF MAKING OXIDATION RESISTANT  
AND DUCTILE IRON BASE ALUMINUM ALLOYS**

Walter E. Jominy, Detroit, and Amedee Roy, Ferndale, Mich., assignors to Chrysler Corporation, Highland Park, Mich., a corporation of Delaware  
No Drawing. Original application Apr. 26, 1957, Ser. No. 655,191, now Patent No. 3,059,326, dated Oct. 23, 1962. Divided and this application Apr. 17, 1961, Ser. No. 103,257

**12 Claims. (Cl. 148—3)**

The present application is a division of our copending application Serial No. 655,191, filed April 26, 1957, now Patent No. 3,059,326, granted October 23, 1962.

This invention relates to methods for making metal bodies and products constituted of ferrous based alloys having substantial oxidation resistance and fortified for use in high temperature environments. The invention is especially directed to methods for making ferrous alloy bodies of this character possessed of a core body structure and an integral casing layer in both of which iron and aluminum are the predominant ingredients and which bodies possess sufficient ductility in at least one stage of their constitution to facilitate their cold and/or hot working by conventional procedures. More specifically the invention concerns methods for making metal bodies composed of an alloy core essentially consisting of iron and aluminum in solid solution and an external integral casing or facing consisting essentially of compounds of iron and aluminum. The invention also concerns a welding process utilizing a welding rod which is of the core body composition of the invention.

Recent developments in the field of gas turbine engines have created a need for alloys capable of withstanding high temperatures and which have sufficient room temperature ductility to facilitate fabrication. Especially desirable are alloys having excellent oxidation resistance under continuous periods of high temperature service and under operations producing thermal shock occasioned by cyclic heating and cooling. As an example of these needs, consider a gas turbine burner liner. It must be made of metal that can be formed to shape and machined. In use it will normally be exposed for substantial periods, to temperatures in the range of about 1600° F. to 2400° F. during operation of the turbine engine. Presently available are only expensive and strategic alloys moderately satisfactory for this application and the problem is therefore to provide a suitable low cost satisfactory alloy structure for this and other applications where one or more of the stated conditions exist.

The substantial heat resistance of certain iron-aluminum alloys with their low content of strategic and expensive raw materials make them attractive. However, experience has indicated that there is a correlation between the oxidation resistance of iron-aluminum alloys and their aluminum content, and between the ductility of iron-aluminum alloys at room temperature and their aluminum content and that a gradual decrease in ductility and increase in heat resistance is normally associated with increased concentration of aluminum in the alloy.

Unfortunately, one of the basic difficulties with iron-aluminum alloys having substantial heat and oxidation resistance is their lack of adequate ductility at room temperature essential to their cold and/or hot working in rolling, forming, bending, and forging operations. Thus our investigations have indicated, for example, that binary iron-aluminum alloys conventionally prepared under slag conditions or in an inert atmosphere and containing about 10% by weight and more of aluminum lack adequate room temperature fabricability, i.e., they have less than 5% elongation by standard room temperature tensile

2

testing are brittle and difficult to process. This is even true at times with respect to iron-aluminum alloy compositions containing between about 8 to 10% by weight of aluminum depending upon processing and heat treatment or when these alloys contain carbon or other alloying elements or dissolved gases. In any event unless specially processed, compositions containing aluminum in this range and greater will have insufficient ductility needed for cold working. At least about 10% and in many cases 20% elongation on standard tensile testing specimens at room temperature is required for this purpose. Moreover, it has been found that lack of ductility is an inherent characteristic in ferrous compositions having sufficient aluminum for substantially continuous periods of protection against severe oxidation at elevated temperatures. For instance, at least 8% aluminum is required in the alloy for a temperature of 1800° F. and about 16% aluminum at 2200° F.

Some attempts have been made to reduce the room temperature brittleness of the iron-aluminum alloy products by producing the alloy composition under vacuum melt conditions and this has resulted primarily in some improvement in hot rolling. Efforts to combine with this procedure a reduction in oxygen impurities by adding carbon to the alloy to combine with the oxygen impurities in the melt and give off carbon dioxide or by passing hydrogen through the melt to combine with the oxygen impurities to form water vapor has produced some further improvement in ductility. These procedures are, however, expensive and time consuming. Moreover, cold working is adversely affected by carbon additions especially above 0.03% by weight and where the aluminum content is above about 12% by weight the percentage elongation of the specimens under room temperature tensile tests is generally insufficient for cold working at room temperature, i.e., is below 10% elongation depending upon the specific procedure employed. Thus a 14% iron-aluminum alloy made by vacuum melting procedures will have good oxidation resistance up to 2200° F. for long periods of time but will only have about a 5% elongation at room temperature.

We have made the surprising discovery that the aforesaid problems may be overcome and oxidation and corrosion resistant metal refractory bodies and products of alloys of iron and aluminum useful for high temperature service over long periods of time and having in at least one stage of their making, sufficient elongation at room temperature for hot and cold rolling, may be obtained by a unique process involving initially compounding the body of iron-aluminum alloy using conventional melt procedures with a relatively low content of aluminum, preferably between about 3½% to 8% of aluminum, normally insufficient to render it effectively oxidation resistant above about 1800° F. and then coating the exterior of the alloy body with a layer or film of pure or substantially pure metallic aluminum or alloys rich in aluminum, as by spraying, dipping, or other coating procedures, utilizing a suitable flux wherever necessary, and then preferably subjecting the aluminum coated iron-aluminum body in use or preferably prior thereto to a diffusion anneal treatment at a relatively low temperature, in the order of about 1300° F. to 1600° F. for a suitable period, for example, between about one to about three hours.

According to our invention, the aluminum coating provides in combination with the iron-aluminum core body an integral iron-aluminum alloy structure having a facial casing portion or strata high in aluminum which will adapt it for long service exposure at high temperatures and which will have the equivalent oxidation resistance of an iron-aluminum alloy having for instance as much as

16% and more aluminum content. Its outstanding refractory properties at elevated temperatures is evident from oxidation tests made at temperatures ranging from 1800° F. to 2400° F. for periods up to 300 hours without any indication of deleterious damage to the alloy structure or its exposed surface. Moreover, prior to coating, the iron-aluminum core body will have good room temperature ductility as evident from elongations of 15 to 35% at room temperature under conventional tensile tests and therefore may be readily cold and hot worked. It will, of course, be understood that the coated structures may be slightly worked after coating but will not be nearly as ductile. In fact, they may be brittle, as the coating, depending upon its thickness, will be capable of only limited deformation. The thicker the coating the less deformation is possible. It is therefore preferred that any forming, machining or other operations be performed prior to coating so that the full benefit thereof may be obtained in subsequent use.

The exact nature of what occurs in the coated structure to produce the foregoing excellent results is not exactly known, but some idea may be had from a comparison of what is believed to occur upon aluminum coating and heat treating an ordinary iron or plain carbon steel core with a similarly coated core of iron-aluminum alloy. In the first case the pure aluminum and compounds of iron and aluminum such as  $FeAl_3$ ,  $FeAl$ , and  $Fe_3Al$  believed to constitute the composition of the outer layer are believed upon heating to diffuse inwardly to completely combine, for all practical purposes, with the iron core material to form solid solutions of aluminum and iron and produce surface areas of aluminum oxide that will slag away with iron oxide after short periods of exposure at temperatures above 1800° F. Stated otherwise, rapid oxidation occurs. In the second case where in accordance with the present invention, the core is an iron-aluminum alloy, preferably containing at least about 3½% by weight of aluminum in solid solution with the iron of this core and the aluminum is in sufficient amount that it tends to resist and retard the migration of the pure aluminum and iron-aluminum compounds of the surface coating into the body to form solid solutions of iron and aluminum. These surface compounds which contain as much as 50% (atomic weight) and more aluminum therefore remain to protect the structure from rapid oxidation at high temperatures. Moreover, after these compounds are all used up by oxidation over extended exposures, there will still be at the surface the solid solutions of iron and aluminum of the core structure or that formed following coating and although these solid solutions are not believed as resistant to oxidation as the aluminum compounds they will nevertheless provide considerable protection.

In some instances as where severe oxidation conditions at high temperatures are anticipated, our invention may utilize a core body made by conventional melt procedures using greater amounts of aluminum than will provide ductility but preferably using the vacuum melt procedures referred to above in order to start with a core material of ductile character higher in aluminum than conventionally possible, in either event to obtain by means of the iron-aluminum surface compounds even greater oxidation resistance than described above for alloys having such percentages of aluminum. Furthermore, some of the novel benefits of our invention may also be obtained by recoating with aluminum and heat treating a core of iron previously coated with aluminum and heat treated, so as to provide in effect an under surface of a solid solution of iron and aluminum as a surface repellent barrier to the aluminum compounds produced by the second coating.

Accordingly, it is the principal object of our invention to provide aluminum coated ferrous based aluminum alloy bodies characterized by oxidation resistance at relatively high temperature in the order of 1600° F. to 2400°

F. and that have sufficient room temperature ductility in at least one stage of their making to facilitate hot and cold fabrication by conventional procedures.

A related object is to provide a ferrous body comprising pure iron, carbon steel and the like having a surface strata comprising iron and aluminum in solid solution overlaid with compounds of iron and aluminum to render the body resistant to oxidation at high temperatures.

Another object is to provide methods of making iron based aluminum alloy bodies having good oxidation resistance at relatively high temperatures in the order of 1600° F. to 2400° F., having satisfactory cold workability at room temperature in at least one stage of their fabrication and having hot workability at temperatures above 1800° F.

A further object is to provide a novel process for producing iron-aluminum alloy bodies resistant to oxidation at elevated temperatures and possessing sufficient ductility at room temperature at one stage in their fabrication to be cold workable, which comprises making an iron-aluminum alloy core having substantial ductility at room temperature and comprising a solid solution of iron and aluminum, coating the core with metallic aluminum and then effecting heat diffusion of the metallic aluminum of said coating into the surface of said core and outward migration of iron to form iron aluminum compounds high in aluminum at the surface of the body.

A specific object is to provide a metal structure predominantly of iron and aluminum and composed of an iron based alloy body possessed of room temperature ductility and containing relatively small amounts preferably between about 3½ to about 8% by weight of aluminum which body has a surface coating of aluminum diffused therewith to provide with said body a structure having excellent resistance to substantial oxidation and disintegration at elevated temperatures.

A further specific object is to provide an iron-aluminum alloy body as in the preceding object wherein said body contains between about 8 to about 12% aluminum incorporated therein by vacuum melting procedures with or without removal of oxygen impurities.

A related object is to coat with metallic aluminum a ductile iron base-aluminum body containing up to about 12% by weight of aluminum in solid solution with the iron thereof and to heat treat the coated body at a relatively low temperature under about 1500° F. to cause diffusion of the metallic aluminum of the coating into the surface of the alloy body to increase the aluminum concentration of the iron-aluminum at such surface whereby to render the body capable of resisting oxidation at temperatures of above 2200° F.

A further specific object is to provide iron-aluminum alloy bodies capable of substantial oxidation resistance and hot working at elevated temperatures between about 1600° F. and 2400° F. comprising a workable iron-aluminum alloy core containing less than about 16% aluminum but more than about 3% thereof and an exterior iron-aluminum stratum or layer containing above about 20% aluminum by weight and in concentration greater than that of the core.

Still another object is to provide a process for protecting a welded low carbon steel structure that has been aluminized for oxidation protection from destruction of the bond and opening of the joint at the weld at elevated temperatures due to substantial oxidation which comprises welding the joint with a welding rod composed of a ductile iron base-aluminum alloy and thereafter coating the weld with metallic aluminum.

Other objects and advantages of our invention will become more evident from the following description.

According to the present invention, an iron-aluminum alloy body that is of ductile character and that has an elongation of at least about 10% at room temperature may be formed by conventional melting methods so as to

preferably contain between about 3½% to 6% aluminum by weight, and even up to 8% by weight where proper precautions are taken in processing. If made by vacuum melting procedures the aluminum content may be up to about 12% by weight. The alloy body in this ductile condition is then preferably cold or hot worked as desired to predetermined shape and size and machined as needed. It is then coated with an aluminum base material which may be pure metallic aluminum or an aluminum alloy rich in aluminum. Any conventional procedure with or without fluxing may be employed for producing this coating but best results are found to be obtained by employing hot dipping procedures in which the iron-aluminum alloy body to be coated is immersed in a bath of molten aluminum or aluminum alloy at a predetermined temperature for a predetermined length of time sufficient to effect a satisfactory coating thereof.

The aluminum coating treatment may be performed continuously or by means of a batch-type process. The temperature of the bath of molten aluminum or aluminum alloy is subject to considerable variation, a range of 1300° F. to 1500° F. having been found to produce satisfactory results. The period of treatment in the molten bath may vary from a few seconds to an hour depending upon the size of the body or core being treated. The thickness of aluminum coating to be obtained on the core body is not too critical and is preferably in the order of one to ten thousandths of an inch.

Following coating, the treated alloy body is preferably heat treated. In most cases it will be found that a temperature in the order of about 1500° F. for a period of about two hours will suffice. This treatment assures the diffusion of the free aluminum of the coating into the surface of the core to form with migrating iron therein further high melting point iron-aluminum compounds believed to be responsible for the refractory character of the aluminized iron-aluminum alloy body. The heat treatment is believed to increase the case depth or thickness of the protective layer sufficiently to materially improve the oxidation resistance of the body but the depth or thickness is not made so great that the concentration of aluminum in the case or layer is diluted enough to permit substantial impairment of the oxidation resistance of the body at high temperatures. It will be understood that the heat treatment is not limited to the time and temperature given but may be subject to considerable variation in temperature and time. For example if the conditions are right it may take place in actual use, although such is not recommended if the temperature is above 1800° F. as the total oxidation resistance of the body is reduced thereby. The aluminized iron-aluminum alloy body is found to withstand severe oxidation conditions at temperatures above 1600° F. and even as high as 2400° F. and to an extent not possible with aluminum coated plain carbon steels. As previously stated, the exact reason for the improved or beneficial effect of the diffused aluminum coating upon the iron-aluminum base alloy is not fully understood. In addition to reasons already expressed, it is believed that the coating is responsible for producing substantially stable iron-aluminum compounds of high aluminum content and consequently of higher refractory character at the surface. The greater oxidation resistance may also possibly be explained by the fact that the aluminum concentration gradient between the core and the coating is at a much lower value than in the case of aluminized steel and consequently the rate of decomposition of the iron-aluminum compound at the surface and diffusion of the aluminum from the surface at elevated temperatures is appreciably reduced.

Although as pointed out above, small additions of aluminum to substantially pure ferrous bodies or ferrous base alloy bodies appear to improve their oxidation resistance in the aluminized condition, a minimum level of aluminum, over about 3% by weight alloyed with

the ferrous base material is required to develop a refractory alloy resistant to oxidation at temperatures up to about 2400° F. We have found for example by experimentation that an iron-aluminum alloy body containing about 3½% by weight of aluminum and which is aluminum coated and heat treated, has a life in the order of about 50 hours when heated in air at 2200° F. Moreover, the oxidation resistance of such an aluminized body wherein the alloy body contains about 4¼% was found to be considerably better than the 3½% material, but one containing about 5½% aluminum exposed to the same conditions as the 3½% alloy was not damaged at all after a period of more than 300 hours duration.

In the preparation of the iron-aluminum core or body, it is preferred that any carbon alloying content of the alloy be kept as low as possible because it is found that carbon decreases the oxidation resistance of aluminized iron-aluminum alloys. We have also found that a decrease in the room temperature ductility of the iron-aluminum alloy results from an increase of the carbon content above the range of about 0.03% to 0.05%. In general, the effect of alloying additions, other than aluminum to the iron, on the oxidation resistance of iron-aluminum alloy bodies aluminized as described above and upon their other physical properties seems to be that at relatively low levels of alloying content with elements other than aluminum there is only a slight decrease or no appreciable effect on the oxidation resistance of the aluminized iron-aluminum base alloy but at high levels of such alloying with elements other than aluminum the resistance to oxidation appears to be reduced appreciably. The following table presents preferred ranges of alloying additions other than aluminum for the compositions of the invention. It will be understood, however, that the invention is not limited thereto:

|                  | Percent by weight             |
|------------------|-------------------------------|
| Carbon.....      | As low as possible up to 0.5. |
| Silicon.....     | 0-5.                          |
| Titanium.....    | 0-5.                          |
| 40 Chromium..... | 0-25.                         |
| Manganese.....   | 0-30.                         |
| Nickel.....      | 0-30.                         |
| Columbium.....   | 0-7.                          |
| Molybdenum.....  | 0-10.                         |
| 45 Tungsten..... | 0-10.                         |
| Vanadium.....    | 0-10.                         |
| Cobalt.....      | 0-20.                         |
| Copper.....      | 0-3.                          |
| Zirconium.....   | 0-5.                          |

Not only does the aluminum alloying of the ferrous body improve its oxidation and scale resistance in the aluminized condition, but such also protects welds in the body from destruction by substantial oxidation during exposure at high temperatures. Deterioration of the weld has heretofore been experienced after 100 hours of exposure with steel structures welded with conventional welding rods or by simple "Heliarc" joining and then coated with aluminum. Where steel pieces to be welded and aluminum dipped were welded using a welding rod made from the iron-aluminum compositions of our invention, for instance an iron-aluminum alloy containing about 6% aluminum, as the electrode, the use of such rod has successfully prevented oxidation of the welded area. An aluminum coated welded area of this kind when exposed to oxidation at a temperature of 1700° F. showed no oxidation after 300 hours whereas a weld made with stainless steel and similarly heated for only 240 hours showed very definite scale and oxidation and showed the presence of black oxide after only 100 hours of exposure. The aluminum content of the welding rod alloy composition will be at least about 3% by weight preferably at least about 6% by weight and the aluminum coated welded area will be preferably heat treated as described above with regard to the composition products made by this invention.

A fuller understanding of the invention and its further objects and advantages will be had from the following examples of specific metal structures and of typical processes by which they may be produced. Such examples are intended only for illustration of the invention and not as a limitation upon its scope. Wherever in the following examples reference is made to tensile testing such tests were made in accordance with standard ASTM practice and at room temperature.

*Example I*

An alloy composition of iron and aluminum was prepared under an Argon atmosphere by melting, by induction heating in a magnesia crucible, 1780 grams of electrolytic iron after which 120 grams of commercial 2S aluminum was added to the molten iron and stirred thoroughly therein. The molten alloy containing approximately 6% by weight of aluminum was then poured into an investment mold assembly comprising several tensile test bars and one  $\frac{3}{4}$ " round bar.

The  $\frac{3}{4}$ " alloy bar was then sectioned into slugs and machined to 0.70" diameter and 0.250" long. The machined slugs were then degreased in a trichlorethylene bath and coated with any conventional flux such as "Alcoa" No. 33 flux and preferably a flux such as described in the copending application of Walter E. Jominy et al., Serial No. 344,190, filed March 23, 1953. The slugs were then aluminum-coated by hot dipping them into a bath of commercial 2S aluminum maintained at a temperature of 1350° F. and held in the bath for a period of two minutes after which they were removed. The coated slugs were then diffusion annealed at a temperature of 1500° F. for two hours.

Oxidation tests were carried out on the samples in still air in a furnace held at a predetermined temperature. Duplicate samples were tested at temperatures ranging from 1800° F. to 2500° F. Weight change measurements as well as visual observations were made at regular intervals during the testing. From this testing and observations it was apparent that the coated alloy would incur no damage whatever in oxidation tests when the material was tested 1800° F. for 200 hours, at 2000° F. for 300 hours, and at 2400° F. for 240 hours. The mechanical properties of the alloy were measured at room temperature and at 1350° F. Conventional tensile tests at room temperature prior to coating indicated that the ductility of the alloy was good and averaged 27% elongation in the samples. The alloy made herein contained a nominal 6% aluminum by weight and 5.65% aluminum by analysis.

*Example II*

An alloy of iron and aluminum was prepared from commercial grade materials employing the same procedure as described with respect to Example I using in this instance SAE 1010 steel as the base material and 2S aluminum. The alloy made in accordance with this example upon testing showed substantial oxidation resistance but was somewhat lower than that for the alloy of Example I at extremely high temperatures. Moreover this alloy was relatively brittle in the cast condition at room temperature and its elongation was 0.5%.

*Example III*

An alloy was prepared as in Example No. I using Armco iron as the base material. Upon testing this material prior to coating it was found to be very ductile. It had an elongation of between 16 to 20% by room temperature tensile testing. Moreover after aluminum coating this alloy was found to withstand severe oxidation conditions at elevated temperatures and was substantially equal to the alloy of Example I in this characteristic.

*Example IV*

An iron base aluminum alloy was prepared in accord-

5  
8  
5  
ance with the procedure of Example I using the same base and alloying materials but employing 1% of aluminum by weight. The oxidation resistance of this alloy structure was good for 53 hours at 2000° F. and 25 hours at 2200° F. The material was very ductile.

*Example V*

An alloy structure was prepared in accordance with the procedure of Example I using the same base and alloying materials but wherein the percentage by weight of aluminum was 2%. The oxidation resistance of this structure was good for 95 hours at 2000° F., 25 hours at 2200° F. and 20 hours at 2400° F. The material had an elongation of 35 to 40% under short time tensile testing at room temperature.

*Example VI*

An alloy structure was prepared as in Example I differing in using 3% aluminum. The oxidation resistance of this structure was good for 95 hours at 2000° F., 25 hours at 2200° F., and 20 hours at 2400° F. The material had an elongation of 40 to 42% by tensile testing at room temperature prior to coating.

*Example VII*

An alloy structure was prepared in accordance with Example No. I employing 4% aluminum. The oxidation resistance of this material was good for 95 hours at 2000° F., 50 hours at 2200° F., and 20 hours at 2400° F. The material had an elongation of 33 to 35% by tensile testing at room temperature prior to coating.

*Example VIII*

An alloy structure was prepared in accordance with Example No. I using 5% aluminum by weight. Oxidation tests indicated no damage to the samples after 225 hours at 2000° F. The material had an elongation of 28 to 30% by tensile testing at room temperature prior to coating.

*Example IX*

An alloy structure was prepared in accordance with the procedure of Example I using 8% aluminum. On oxidation testing the material exhibited no damage at 2000° F. after 300 hours, at 2200° F. after 240 hours, at 2400° F. after 265 hours, and 2500° F. after 100 hours. The material had an elongation of between 5 to 20% by tensile tests at room temperature.

*Example X*

An alloy structure was prepared in accordance with the procedure of Example No. I using 10% aluminum. On oxidation testing this alloy structure exhibited no damage upon testing at 2200° F. for 240 hours, at 2400° F. after 265 hours, and at 2500° F. after 100 hours. The material had an elongation of between 1 to 3% by tensile testing at room temperature prior to coating.

*Example XI*

An alloy structure was made in accordance with the procedure of Example I using 14% aluminum. Upon oxidation testing the structure showed no damage after testing at 2400° F. for 265 hours and at 2500° F. after 100 hours. The structure had an elongation of less than 1% by tensile testing at room temperature prior to coating.

*Example XII*

An alloy structure as described in Example X was made by vacuum melt procedures to obtain greater ductility at room temperature.

*Example XIII*

5  
70  
75  
76  
77  
78  
79  
80  
81  
82  
83  
84  
85  
86  
87  
88  
89  
90  
91  
92  
93  
94  
95  
96  
97  
98  
99  
100  
101  
102  
103  
104  
105  
106  
107  
108  
109  
110  
111  
112  
113  
114  
115  
116  
117  
118  
119  
120  
121  
122  
123  
124  
125  
126  
127  
128  
129  
130  
131  
132  
133  
134  
135  
136  
137  
138  
139  
140  
141  
142  
143  
144  
145  
146  
147  
148  
149  
150  
151  
152  
153  
154  
155  
156  
157  
158  
159  
160  
161  
162  
163  
164  
165  
166  
167  
168  
169  
170  
171  
172  
173  
174  
175  
176  
177  
178  
179  
180  
181  
182  
183  
184  
185  
186  
187  
188  
189  
190  
191  
192  
193  
194  
195  
196  
197  
198  
199  
200  
201  
202  
203  
204  
205  
206  
207  
208  
209  
210  
211  
212  
213  
214  
215  
216  
217  
218  
219  
220  
221  
222  
223  
224  
225  
226  
227  
228  
229  
230  
231  
232  
233  
234  
235  
236  
237  
238  
239  
240  
241  
242  
243  
244  
245  
246  
247  
248  
249  
250  
251  
252  
253  
254  
255  
256  
257  
258  
259  
259  
260  
261  
262  
263  
264  
265  
266  
267  
268  
269  
270  
271  
272  
273  
274  
275  
276  
277  
278  
279  
280  
281  
282  
283  
284  
285  
286  
287  
288  
289  
290  
291  
292  
293  
294  
295  
296  
297  
298  
299  
300  
301  
302  
303  
304  
305  
306  
307  
308  
309  
310  
311  
312  
313  
314  
315  
316  
317  
318  
319  
320  
321  
322  
323  
324  
325  
326  
327  
328  
329  
330  
331  
332  
333  
334  
335  
336  
337  
338  
339  
339  
340  
341  
342  
343  
344  
345  
346  
347  
348  
349  
349  
350  
351  
352  
353  
354  
355  
356  
357  
358  
359  
359  
360  
361  
362  
363  
364  
365  
366  
367  
368  
369  
369  
370  
371  
372  
373  
374  
375  
376  
377  
378  
379  
379  
380  
381  
382  
383  
384  
385  
386  
387  
388  
389  
389  
390  
391  
392  
393  
394  
395  
396  
397  
398  
399  
399  
400  
401  
402  
403  
404  
405  
406  
407  
408  
409  
409  
410  
411  
412  
413  
414  
415  
416  
417  
418  
419  
419  
420  
421  
422  
423  
424  
425  
426  
427  
428  
429  
429  
430  
431  
432  
433  
434  
435  
436  
437  
438  
439  
439  
440  
441  
442  
443  
444  
445  
446  
447  
448  
449  
449  
450  
451  
452  
453  
454  
455  
456  
457  
458  
459  
459  
460  
461  
462  
463  
464  
465  
466  
467  
468  
469  
469  
470  
471  
472  
473  
474  
475  
476  
477  
478  
479  
479  
480  
481  
482  
483  
484  
485  
486  
487  
488  
489  
489  
490  
491  
492  
493  
494  
495  
496  
497  
498  
499  
499  
500  
501  
502  
503  
504  
505  
506  
507  
508  
509  
509  
510  
511  
512  
513  
514  
515  
516  
517  
518  
519  
519  
520  
521  
522  
523  
524  
525  
526  
527  
528  
529  
529  
530  
531  
532  
533  
534  
535  
536  
537  
538  
539  
539  
540  
541  
542  
543  
544  
545  
546  
547  
548  
549  
549  
550  
551  
552  
553  
554  
555  
556  
557  
558  
559  
559  
560  
561  
562  
563  
564  
565  
566  
567  
568  
569  
569  
570  
571  
572  
573  
574  
575  
576  
577  
578  
579  
579  
580  
581  
582  
583  
584  
585  
586  
587  
588  
589  
589  
590  
591  
592  
593  
594  
595  
596  
597  
598  
599  
599  
600  
601  
602  
603  
604  
605  
606  
607  
608  
609  
609  
610  
611  
612  
613  
614  
615  
616  
617  
618  
619  
619  
620  
621  
622  
623  
624  
625  
626  
627  
628  
629  
629  
630  
631  
632  
633  
634  
635  
636  
637  
638  
639  
639  
640  
641  
642  
643  
644  
645  
646  
647  
648  
649  
649  
650  
651  
652  
653  
654  
655  
656  
657  
658  
659  
659  
660  
661  
662  
663  
664  
665  
666  
667  
668  
669  
669  
670  
671  
672  
673  
674  
675  
676  
677  
678  
679  
679  
680  
681  
682  
683  
684  
685  
686  
687  
688  
689  
689  
690  
691  
692  
693  
694  
695  
696  
697  
698  
699  
699  
700  
701  
702  
703  
704  
705  
706  
707  
708  
709  
709  
710  
711  
712  
713  
714  
715  
716  
717  
718  
719  
719  
720  
721  
722  
723  
724  
725  
726  
727  
728  
729  
729  
730  
731  
732  
733  
734  
735  
736  
737  
738  
739  
739  
740  
741  
742  
743  
744  
745  
746  
747  
748  
749  
749  
750  
751  
752  
753  
754  
755  
756  
757  
758  
759  
759  
760  
761  
762  
763  
764  
765  
766  
767  
768  
769  
769  
770  
771  
772  
773  
774  
775  
776  
777  
778  
779  
779  
780  
781  
782  
783  
784  
785  
786  
787  
788  
789  
789  
790  
791  
792  
793  
794  
795  
796  
797  
798  
799  
799  
800  
801  
802  
803  
804  
805  
806  
807  
808  
809  
809  
810  
811  
812  
813  
814  
815  
816  
817  
818  
819  
819  
820  
821  
822  
823  
824  
825  
826  
827  
828  
829  
829  
830  
831  
832  
833  
834  
835  
836  
837  
838  
839  
839  
840  
841  
842  
843  
844  
845  
846  
847  
848  
849  
849  
850  
851  
852  
853  
854  
855  
856  
857  
858  
859  
859  
860  
861  
862  
863  
864  
865  
866  
867  
868  
869  
869  
870  
871  
872  
873  
874  
875  
876  
877  
878  
879  
879  
880  
881  
882  
883  
884  
885  
886  
887  
888  
889  
889  
890  
891  
892  
893  
894  
895  
896  
897  
898  
899  
899  
900  
901  
902  
903  
904  
905  
906  
907  
908  
909  
909  
910  
911  
912  
913  
914  
915  
916  
917  
918  
919  
919  
920  
921  
922  
923  
924  
925  
926  
927  
928  
929  
929  
930  
931  
932  
933  
934  
935  
936  
937  
938  
939  
939  
940  
941  
942  
943  
944  
945  
946  
947  
948  
949  
949  
950  
951  
952  
953  
954  
955  
956  
957  
958  
959  
959  
960  
961  
962  
963  
964  
965  
966  
967  
968  
969  
969  
970  
971  
972  
973  
974  
975  
976  
977  
978  
979  
979  
980  
981  
982  
983  
984  
985  
986  
987  
988  
989  
989  
990  
991  
992  
993  
994  
995  
996  
997  
998  
999  
999  
1000  
1001  
1002  
1003  
1004  
1005  
1006  
1007  
1008  
1009  
1009  
1010  
1011  
1012  
1013  
1014  
1015  
1016  
1017  
1018  
1019  
1019  
1020  
1021  
1022  
1023  
1024  
1025  
1026  
1027  
1028  
1029  
1029  
1030  
1031  
1032  
1033  
1034  
1035  
1036  
1037  
1038  
1039  
1039  
1040  
1041  
1042  
1043  
1044  
1045  
1046  
1047  
1048  
1049  
1049  
1050  
1051  
1052  
1053  
1054  
1055  
1056  
1057  
1058  
1059  
1059  
1060  
1061  
1062  
1063  
1064  
1065  
1066  
1067  
1068  
1069  
1069  
1070  
1071  
1072  
1073  
1074  
1075  
1076  
1077  
1078  
1079  
1079  
1080  
1081  
1082  
1083  
1084  
1085  
1086  
1087  
1088  
1089  
1089  
1090  
1091  
1092  
1093  
1094  
1095  
1096  
1097  
1098  
1099  
1099  
1100  
1101  
1102  
1103  
1104  
1105  
1106  
1107  
1108  
1109  
1109  
1110  
1111  
1112  
1113  
1114  
1115  
1116  
1117  
1118  
1119  
1119  
1120  
1121  
1122  
1123  
1124  
1125  
1126  
1127  
1128  
1129  
1129  
1130  
1131  
1132  
1133  
1134  
1135  
1136  
1137  
1138  
1139  
1139  
1140  
1141  
1142  
1143  
1144  
1145  
1146  
1147  
1148  
1149  
1149  
1150  
1151  
1152  
1153  
1154  
1155  
1156  
1157  
1158  
1159  
1159  
1160  
1161  
1162  
1163  
1164  
1165  
1166  
1167  
1168  
1169  
1169  
1170  
1171  
1172  
1173  
1174  
1175  
1176  
1177  
1178  
1179  
1179  
1180  
1181  
1182  
1183  
1184  
1185  
1186  
1187  
1188  
1189  
1189  
1190  
1191  
1192  
1193  
1194  
1195  
1196  
1197  
1198  
1199  
1199  
1200  
1201  
1202  
1203  
1204  
1205  
1206  
1207  
1208  
1209  
1209  
1210  
1211  
1212  
1213  
1214  
1215  
1216  
1217  
1218  
1219  
1219  
1220  
1221  
1222  
1223  
1224  
1225  
1226  
1227  
1228  
1229  
1229  
1230  
1231  
1232  
1233  
1234  
1235  
1236  
1237  
1238  
1239  
1239  
1240  
1241  
1242  
1243  
1244  
1245  
1246  
1247  
1248  
1249  
1249  
1250  
1251  
1252  
1253  
1254  
1255  
1256  
1257  
1258  
1259  
1259  
1260  
1261  
1262  
1263  
1264  
1265  
1266  
1267  
1268  
1269  
1269  
1270  
1271  
1272  
1273  
1274  
1275  
1276  
1277  
1278  
1279  
1279  
1280  
1281  
1282  
1283  
1284  
1285  
1286  
1287  
1288  
1289  
1289  
1290  
1291  
1292  
1293  
1294  
1295  
1296  
1297  
1298  
1299  
1299  
1300  
1301  
1302  
1303  
1304  
1305  
1306  
1307  
1308  
1309  
1309  
1310  
1311  
1312  
1313  
1314  
1315  
1316  
1317  
1318  
1319  
1319  
1320  
1321  
1322  
1323  
1324  
1325  
1326  
1327  
1328  
1329  
1329  
1330  
1331  
1332  
1333  
1334  
1335  
1336  
1337  
1338  
1339  
1339  
1340  
1341  
1342  
1343  
1344  
1345  
1346  
1347  
1348  
1349  
1349  
1350  
1351  
1352  
1353  
1354  
1355  
1356  
1357  
1358  
1359  
1359  
1360  
1361  
1362  
1363  
1364  
1365  
1366  
1367  
1368  
1369  
1369  
1370  
1371  
1372  
1373  
1374  
1375  
1376  
1377  
1378  
1379  
1379  
1380  
1381  
1382  
1383  
1384  
1385  
1386  
1387  
1388  
1389  
1389  
1390  
1391  
1392  
1393  
1394  
1395  
1396  
1397  
1398  
1399  
1399  
1400  
1401  
1402  
1403  
1404  
1405  
1406  
1407  
1408  
1409  
1409  
1410  
1411  
1412  
1413  
1414  
1415  
1416  
1417  
1418  
1419  
1419  
1420  
1421  
1422  
1423  
1424  
1425  
1426  
1427  
1428  
1429  
1429  
1430  
1431  
1432  
1433  
1434  
1435  
1436  
1437  
1438  
1439  
1439  
1440  
1441  
1442  
1443  
1444  
1445  
1446  
1447  
1448  
1449  
1449  
1450  
1451  
1452  
1453  
1454  
1455  
1456  
1457  
1458  
1459  
1459  
1460  
1461  
1462  
1463  
1464  
1465  
1466  
1467  
1468  
1469  
1469  
1470  
1471  
1472  
1473  
1474  
1475  
1476  
1477  
1478  
1479  
1479  
1480  
1481  
1482  
1483  
1484  
1485  
1486  
1487  
1488  
1489  
1489  
1490  
1491  
1492  
1493  
1494  
1495  
1496  
1497  
1498  
1499  
1499  
1500  
1501  
1502  
1503  
1504  
1505  
1506  
1507  
1508  
1509  
1509  
1510  
1511  
1512  
1513  
1514  
1515  
1516  
1517  
1518  
1519  
1519  
1520  
1521  
1522  
1523  
1524  
1525  
1526  
1527  
1528  
1529  
1529  
1530  
1531  
1532  
1533  
1534  
1535  
1536  
1537  
1538  
1539  
1539  
1540  
1541  
1542  
1543  
1544  
1545  
1546  
1547  
1548  
1549  
1549  
1550  
1551  
1552  
1553  
1554  
1555  
1556  
1557  
1558  
1559  
1559  
1560  
1561  
1562  
1563  
1

by weight was then forged at 1800° F. down to  $\frac{3}{4}$ " slab. The slab was then further reduced down to a sheet of a thickness of 0.080" by hot and then cold rolling. This sheet material was then used in the fabrication of gas burner liners, the joint of the liners being welded by "Heliarc" welding using welding rods made from the parent metal forming the sheet as a filler. The gas burner liners were cold formed at room temperature prior to coating by conventional methods. Ample ductility was present for the operation. The liners were then aluminum coated as described in Example No. I and then both liner and weld subjected to oxidation testing at temperatures up to 2400° F. The weld was tested, for example, for 325 hours at 2000° F. without any sign of damage. This was also true under more sever oxidizing conditions. The liner was also tested in actual use in a turbine engine and after many hours of operation showed no deterioration from oxidation at the high temperature prevailing.

It is obvious that many variations may be made in the products and processes of this invention without departing from the spirit and scope thereof as defined in the appended claims.

We claim:

1. A process for producing ferrous base products capable of substantial resistance to oxidation and scaling upon exposure to high temperatures in the order of 1600° F. to 2400° F. comprising casting a metal body consisting essentially of iron and aluminum in solid solution, said body having a substantially uniform aluminum concentration throughout between 3% to 12% by weight of said body and said body being cold workable at room temperature, coating the surface of said body with metal consisting essentially of aluminum and heating said aluminum coated body to increase the aluminum concentration of the iron-aluminum at such surface.

2. A process of producing ferrous base products capable of substantial resistance to oxidation and scaling upon exposure to high temperatures in the order of 1600° F. to 2400° F. comprising casting a metal body consisting essentially of iron and aluminum in solid solution, said aluminum constituting between 3% to 12% by weight of said body and said body being cold workable at room temperatures, coating said body with molten metal consisting essentially of aluminum, and diffusion annealing said coated body at a temperature between about 1300° F. to 1800° F.

3. A process of producing ferrous base products capable of substantial resistance to oxidation and scaling upon exposure to high temperatures in the order of 1600° F. to 2400° F. comprising casting a metal body consisting essentially of iron and aluminum in solid solution, said aluminum constituting between about 3½% to 8% by weight of said body and said body being cold workable at room temperature, coating said body with a metal consisting essentially of aluminum and heat treating said coated body at a temperature between about 1300° F. to 1800° F. for about one to three hours to effect a diffusion anneal thereof.

4. A process of producing ferrous base products capable of substantial resistance to oxidation and scaling upon exposure to high temperatures in the order of 1600° F. to 2400° F. comprising casting a metal body consisting essentially of iron and aluminum in solid solution, said aluminum constituting between about 3% to 12% by weight of said body and said body being cold workable at room temperature, working said body to predetermined size and shape, and then coating said worked body with a layer consisting essentially of aluminum.

5. A process of producing ferrous base products capable of substantial resistance to oxidation and scaling upon exposure to high temperatures in the order of 1600° F. to 2400° F., comprising providing a metal body consisting essentially of iron and aluminum in solid solution, said aluminum constituting between about 3% to 12% by weight of said body, but not in excess of an amount pro-

5 ducing less than 10% elongation by standard tensile testing at room temperature and facilitating cold working of said body at room temperature, working said body to predetermined size and shape, then immersion treating said worked body in a molten composition consisting essentially of aluminum to produce a surface strata of aluminum and compounds of iron and aluminum containing at least about 20% by weight of aluminum and heating said treated body to increase the extent of said last-mentioned 10 iron-aluminum compounds.

6. A process of producing ferrous base products capable of substantial resistance to oxidation and scaling upon exposure to high temperatures in the order of 1600° F. to 2400° F., comprising making a melt from metallic ingredients consisting essentially of iron and aluminum, the latter in amount between about 3% to 12% by weight of said melt, forming a solid body from said melt in which said ingredients are in solid solution said body being cold workable at room temperature, working said solid body to predetermined size and shape, then treating the surface of said solid body with molten metal consisting essentially of aluminum to form compounds of iron and aluminum adjacent the surface of said body containing at least about 20% by weight of aluminum, and diffusion annealing said treated body to increase the extent of said last-mentioned compounds.

7. A process of producing ferrous base products capable of substantial resistance to oxidation and scaling upon exposure to high temperatures in the order of 1600° F. to 2400° F. comprising, vacuum melting a plurality of metallic ingredients consisting essentially of iron and between about 8% to 12% aluminum, casting a solid body from said melt in which said ingredients are in solid solution said body being cold workable at room temperature, 30 working said solid body to predetermined size and shape, then coating said body with molten metal consisting essentially of aluminum and diffusion annealing said coated body.

8. A process as claimed in claim 5 wherein the aluminum content is between about 5½% to 8%.

9. A process as claimed in claim 5 wherein the body includes carbon in amount less than 0.05% by weight.

10. A process as claimed in claim 6 wherein said melt includes ingredients selected from the group consisting of the following elements and mixtures thereof within the limits of each set forth:

|               | Percent by weight |
|---------------|-------------------|
| Carbon        | 0-0.5             |
| Silicon       | 0-5               |
| Titanium      | 0-5               |
| Chromium      | 0-25              |
| Manganese     | 0-30              |
| Nickel        | 0-30              |
| Columbium     | 0-7               |
| 55 Molybdenum | 0-10              |
| Tungsten      | 0-10              |
| Vanadium      | 0-10              |
| Cobalt        | 0-20              |
| Copper        | 0-3               |
| 60 Zirconium  | 0-5               |

11. In a method of welding a joint between two ferrous bodies the improvement which will impart to the joint substantial resistance to oxidation and scaling consisting in welding said bodies at said joint using an alloy welding rod of substantially homogeneous character consisting essentially of iron and between 3½% to 12% aluminum in solid solution and following welding coating the welded area with a metal consisting essentially of aluminum.

12. In the process of producing ductile carbon containing iron-aluminum alloys for producing ferrous base products capable of substantial resistance to oxidation and scaling upon exposure to high temperature, the improvement which consists in making the alloy melt with between about 3% to 12% by weight of aluminum con-

trolling the carbon content of the said melt to an amount no greater than about 0.05% by weight, casting said alloy into an ingot, reducing said ingot to sheet form, cold forming said sheet at room temparture into a product of predetermined shape, coating said product with a continuous layer of aluminum and subsequently subjecting said coated product to heating at a temperature under about 1800° F. sufficient to cause diffusion of the metallic aluminum into the surface of said product.

|              |       |                |       |           |
|--------------|-------|----------------|-------|-----------|
| 2,048,526    | 7/36  | Vander Pyl     | ----- | 148-6     |
| 2,060,765    | 11/36 | Welch          | ----- | 148-127 X |
| 2,140,238    | 12/38 | Leitner        | ----- | 75-124 X  |
| 2,243,979    | 6/41  | Reynolds       | ----- | 29-527    |
| 5 2,303,869  | 12/42 | Quinlan        | ----- | 29-196.2  |
| 2,304,666    | 12/42 | Sturges        | ----- | 29-527    |
| 2,481,962    | 9/49  | Whitfield      | ----- | 117-114   |
| 2,738,289    | 3/56  | Hodge          | ----- |           |
| 2,801,942    | 8/57  | Nachman et al. | ----- | 75-124 X  |
| 10 2,830,922 | 4/58  | Ahles          | ----- | 75-124    |
| 2,851,387    | 9/58  | Low            | ----- | 148-6     |
| 2,930,690    | 3/60  | Meinen         | ----- | 75-129    |

## References Cited by the Examiner

## UNITED STATES PATENTS

1,165,920 12/15 Uyeno.

1,346,062 7/20 Ruder.

1,904,107 4/33 Von Zeerleder 29-196.2

DAVID L. RECK, Primary Examiner.

15 HYLAND BIZOT, ROGER L. CAMPBELL, Examiners.